

## UNITED STATES PATENT OFFICE.

JOHN H. HALL, OF HIGH BRIDGE, NEW JERSEY, ASSIGNOR TO TAYLOR-WHARTON IRON AND STEEL COMPANY, OF HIGH BRIDGE, NEW JERSEY, A CORPORATION OF NEW JERSEY.

## METHOD OF PRODUCING PIPE BALLS.

No Drawing.

Application filed June 5, 1922. Serial No. 566,105.

*To all whom it may concern:*

Be it known that I, JOHN H. HALL, a citizen of the United States, residing at High Bridge, in the county of Hunterdon and State of New Jersey, have invented certain new and useful Improvements in Methods of Producing Pipe Balls, of which the following is a specification.

The object of this invention is to provide for the production of manganese steel pipe balls characterized by their uniformly fine grained structure and by their marked ability to resist the abrasive action of hot skelp.

Heretofore, and before my invention, in making pipe balls of manganese steel, the steel has been poured hot, the effect of which is to dispose the crystals in the form of columns at right angles to the surface of the ball. Moreover, this objectionable and inherently weak crystalline structure is further weakened by burning in the heat treatment of the ball. In service the pressure of the skelp on a ball with this structure weakens the crystal bond and tears apart the columnar structure, thereby impairing, if not actually destroying, the efficiency of the ball.

According to my invention the steel is poured at a temperature close to its freezing point whereby I obtain a casting having a uniformly fine grain structure, and which is further characterized by its freedom from columnar crystals. The avoidance of columnar crystals eliminates burning of the

casting in the heat treatment of the ball. 35 The balls are charged in comparatively small lots into a furnace heated to a temperature of at least 800° C. The temperature is then elevated and brought to about 1060° C. In from twenty-five to forty minutes, whereupon the balls are quenched in water. Practice has demonstrated that a cold-poured ball heated rapidly, in the manner indicated, is remarkable for both its longevity and 40 ability to resist abrasive wear. 45

Having described my invention, I claim:

1. The method of producing pipe balls, which consists in casting balls from manganese steel poured at a temperature close to its freezing point, charging the balls into a 50 hot furnace and rapidly elevating the temperature to about 1060° C. and then quenching the balls.

2. The method of producing pipe balls characterized by their freedom from columnar crystals and by their ability to resist abrasive wear, which consists in charging cold-poured manganese steel balls into a furnace heated to a temperature of at least 800° C., rapidly raising the temperature to 60 the maximum usually employed in the heat treatment of manganese steel, and quenching the balls in water. 55

3. A pipe ball consisting of a cold-poured manganese steel casting free from columnar crystals and burnt spots. 65

In testimony whereof I affix my signature.  
JOHN H. HALL.